

Nov. 15, 1932.

E. C. LOETSCHER

1,887,691

METHOD OF VENEERING

Filed Oct. 8, 1931



Inventor

Emil C. Loetscher.

By  
Harold Howell  
Attorney

## UNITED STATES PATENT OFFICE

EMIL C. LOETSCHER, OF DUBUQUE, IOWA

## METHOD OF VENEERING

Application filed October 8, 1931. Serial No. 567,748.

The object of this invention is to provide an improved method of veneering a base with wood veneer whereby in the finished product the veneer will be practically dent and scratch proof and not subject to disfigurement under ordinary conditions of use by burns from matches, cigarettes and the like laid thereon.

With the above and other objects in view, reference will be had to the accompanying drawing diagrammatically illustrating the parts of one product of the invention juxtaposed for consolidation into a unitary body by a suitable press in the presence of heat.

Referring to the drawing, reference numerals 1 and 2 designate the lower and upper platens respectively of a press such as is usually employed in producing laminated synthetic resin products. The product itself comprises a base 3 which may be solid wood, compound lumber, laminated paper or any other material. In certain products this base is not employed. Upon the base, two layers 4 of paper treated with phenolic condensation product are applied. A single layer may suffice for certain products while others may require three or more layers. A metal plate 5 is next applied and may be aluminum, copper, steel or other metal of high heat conductivity. A layer 6 of paper treated with phenolic condensation product is applied to the metal, and in some instances more than one of these layers may be employed. Wood veneer layer 7, thoroughly saturated with phenolic condensation product is next applied and this wood veneer is preferably a very thin one of approximately  $1/100''$  in thickness. A sheet of tissue or cellophane 8 treated with phenolic condensation product is finally applied, though more than one sheet thereof may be used in certain instances, while in others the tissue or cellophane may not be employed.

Wood veneers have been found to be very susceptible to denting and applicant has discovered that this is due to the fact that under present methods of treating the veneer with phenolic condensation product, many, and probably most, of the microscopic cells or tubes of the wood veneer were not com-

pletely filled with the synthetic product, hence they collapse under pressure and the surface of the wood veneer shows dents. Likewise a sharp object readily digs into the wood veneer and results in scratches. By impregnating the wood veneer under pressure, virtually all of the microscopic cells and tubes thereof are thoroughly filled with phenolic condensation product so that when the latter is reacted the wood of the veneer cannot be compacted or readily penetrated to cause dents or scratches since its cells are completely filled with the hard synthetic product, which in addition to filling the cells of the wood supplies a hard varnish-like surface coating for the wood veneer. These results are not obtainable with wood veneer that has been brush or immersion-coated with the synthetic resin, since in neither of these methods will the synthetic product penetrate much more than the surface portion or cells of the wood veneer.

Pressure impregnation of the wood veneer is accomplished by placing the wood veneer in an air-tight chamber, opening up the cells of the veneer by drawing a vacuum and then flowing the phenolic condensation product into the evacuated chamber without breaking the vacuum. When the chamber is entirely filled with phenolic condensation product, air pressure from 500 to 2,000 pounds per square inch is applied on top of the phenolic condensation product and this, in producing hydrostatic pressure of the same amount on the condensation product, forces the latter into practically all of the cells of the veneer. When such high hydrostatic pressure is used, as 1,000 pounds or more per square inch, the vacuum feature may be dispensed with. In either case, when the air pressure is released, the chamber is opened and the veneer taken out. The wood veneer now has a very different appearance than when merely brush coated or immersed in phenolic condensation product. It has become practically transparent showing that the condensation product has thoroughly penetrated and filled the pores and cellular spaces of the veneer.

Wood veneers, while highly desirable for

table and counter tops and the like, because of the natural beauty of the wood grains, have had to be abandoned in many cases on account of the same not being able to resist 5 disfigurement from such degrees of heat as may be encountered in ordinary use as from hot dishes, lighted matches, cigarettes or the like laid thereon.

Applicant has found that pressure impregnation of the wood veneers, in addition to rendering them dent and scratch proof under ordinary conditions of use, is materially an advance step in making them burn-proof under ordinary conditions of use. In 10 certain cases, pressure impregnation alone answers the purpose, but in others even that failed to make the wood veneers resistant to disfigurement from the effects of certain higher temperatures. Nevertheless, such 15 treatment proved itself to be an advanced step toward perfection in rendering the wood veneer disfigurement proof from the effects of certain high degrees of heat.

Applicant, during the course of experimentation, discovered that if heat is conducted rapidly away from the point of concentration, the pressure impregnated wood veneer would withstand such high temperatures as may be caused by burning matches, cigarettes and hot food dishes laid thereon, without disfigurement. The metal plate 5 lends itself perfectly to the purpose because of its 20 high heat conductivity though it is within the purview of this invention to substitute any 25 other material, as a backing for the phenolic condensation product pressure impregnated wood veneer, that has sufficient heat conductivity as to cause it to disperse, from the point of concentration, heat of a degree that would 30 otherwise injure the wood veneer and damage its surface finish.

Applicant makes no claim to having produced a product that cannot be dented by an excessive blow, as one from a hammer, nor 45 does he claim a product that will be disfigured by excessive heat as that from a blow torch. His product will, however, resist finger pressure without denting, ordinary scratches, and 50 disfigurement from burning matches, cigarettes and even hot dishes. In other words, products made under applicant's method meet all the requirements demanded of furniture, building trim and the like under ordinary usage.

Applicant has further discovered that phenolic condensation product treated tissue, and cellophane when applied to wood veneer increases the burn-resisting qualities of the product and while the same may be adopted, 60 is not essential to the production of a satisfactory burn proof wood veneered article.

As stated, the base 3 may be dispensed with in products calling for decreased thickness.

In eliminating the base 3, a metal plate 5 of 65 increased thickness is adopted, the plate in

this case furnishing the necessary stability. When the base 3 is adopted, the thickness of the metal plate 5 may be reduced to the lowest extent that will enable it to function in the desired heat dispersing degree.

It will be observed that the metal plate 5 is located between two paper layers 4 and 6, either of which may be composed of one or more layers. Various kinds of papers may be used and even textile or felted fabric substituted, but in any event the layers are treated with phenolic condensation product in any desired manner, the essential being that under the influence of heat the paper, due to the fusing of the condensation product with which it is impregnated, will become plastic and adjust itself to the irregularities in the metal plate or layers 3 and 7. If the base 3 is not employed the paper layer or layers 4 on the bottom surface will conform to the contour 80 of the upper face of the press platen 1, or if the base 3 is employed, will conform to that of the upper surface of the base. The upper and lower faces of the paper layers 4 and 6 respectively will conform to the lower and 85 upper faces respectively of the metal plate, and the upper face of the paper layer 6 will conform to the lower face of the wood veneer, permitting the upper veneer to conform to the lower face of the upper press platen 2. In 90 some cases the paper layer 4 as well as the base 3 may be eliminated.

It will be observed that even though the pressure impregnated wood veneer is itself dent-proof, that if backed by a compressible foundation, a severe blow would in certain instances compress the foundation material producing a dent in the same rather than in the wood veneer itself, but since the latter is affixed to the foundation material it would 105 be distorted into the dent made in the foundation material, producing in effect a dent in the wood veneer, though the dent is in the foundation material rather than in the wood veneer. To overcome this, the metal plate 5 as well as the paper layers 4 and 6, which become extremely hard upon the phenolic condensation product therein becoming reacted, provide an armour for the base 3 and 110 prevents the wood veneer from being forced by a severe blow, as may ordinarily be encountered, from forcing the wood veneer into the base 3 and producing in effect a dent in the surface of the wood veneer. It will 115 be apparent that the hard backings 4, 5, 6 if used with wood veneers that are not pressure impregnated, but treated by brushing with or immersing in synthetic resin, will enable the wood veneer itself to be more 120 readily dented since the fibres of the latter being confined between the hard backing and the striking object will readily be compacted and show surface disfigurement which would 125 not be the case were all the cells of the wood 130

veneer completely filled with the synthetic resin as under applicant's method.

In filling the pores or cells of the wood veneer completely with phenolic condensation product by pressure impregnation, the 5 grain of the wood veneer will not rise under certain degrees of heat, and in the case of higher degrees of heat, the grain of the wood veneer will not be raised if the heat, in excess of what pressure impregnation will cause the 10 veneer to withstand, is rapidly carried away from the point of concentration. Raising of the grain of the wood veneer may probably be due to the evaporation of the volatile oil 15 in the natural resins of the wood under the action of heat.

Applicant lays no claim to the production 20 of a product that cannot be dented with a sledge hammer blow or disfigured from the effects of a blow torch flame, but he does 25 claim the production of a product that will withstand the abuses of usage to which furniture, doors, building trim are ordinarily subjected, such as impacts, scratching, and 30 the effects of lighted matches and cigarettes laid thereon.

Obviously both sides of the base 3 may be 35 built up alike, or if the base 3 is not used, a sheet of wood veneer similar to the one 7 40 may take its place with or with, or without the employment of a tissue or cellophane layer similar to the one 8.

Having described the invention, what is 45 claimed as new and useful and desired to be secured by Letters Patent is:

1. The method of making compound lumber having a surface that is dent proof under pressures corresponding to finger nail pressure and proof against burns from heat 40 corresponding to the heat imparted from a lighted cigarette or match when laid thereon, consisting in impregnating the wood veneer in a manner to fill virtually all of the cells thereof with phenolic condensation product, 45 providing for the treated wood veneer a heat-dispersing backing, and subjecting the pack to heat and pressure to react the phenolic condensation product.

2. The method of preventing the raising 50 of the grain of wood veneer of compound lumber from the effects of lighted cigarettes or matches laid thereon, consisting in impregnating the wood veneer in a manner to fill virtually all the cells thereof with 55 phenolic condensation product, providing a metal backing for the treated wood veneer, and in subjecting the pack to heat and pressure to react the phenolic condensation product.

60 3. The method of preventing the raising 65 of the grain of wood veneer of compound lumber from the effects of lighted cigarettes and matches laid thereon, consisting in pressure impregnating the wood veneer with synthetic resin, and in providing a backing there-

for comprising a metal plate between layers of synthetic resin treated material which becomes plastic during the step of reacting the synthetic resin, and in subjecting the pack to heat and pressure to compact the same and react the synthetic resin.

In testimony whereof, I affix my signature.  
EMIL C. LOETSCHER.

75

80

85

90

95

100

105

110

115

120

125

130